

Oct. 3, 1944.

G. HOLST ET AL

2,359,645

ELECTRICAL APPARATUS

Filed Jan. 15, 1941

INSULATING LIQUID CONGEALING  
IN CONTACT WITH AIR AT RATE  
WHICH AUTOMATICALLY SEALS  
CONTAINER LEAKS



INVENTORS:  
GILLES HOLST & CO  
JOHANNES HOEKSTRA  
by *John B. Lemmon*  
ATTORNEY

## UNITED STATES PATENT OFFICE

2,359,645

## ELECTRICAL APPARATUS

Gilles Holst and Johannes Hockstra, Eindhoven,  
Netherlands; vested in the Alien Property Cus-  
todian

Application January 15, 1941, Serial No. 374,560  
In the Netherlands September 6, 1939

1 Claim. (Cl. 174—17)

In electric apparatus such as transformers which are housed in a casing the sealing of this casing is naturally very important, especially if the casing is to be filled with a more or less liquid impregnating material.

Even if careful attention is given to the sealing of the casing there is always the danger that mechanical damage or repeated heating and cooling of the apparatus, may cause small cracks in the casing and leakage of the impregnating material.

The object of the invention is to obviate this difficulty by filling the free space between the casing and the electrical apparatus proper with a viscous electrically insulating material which on exposure to air through leaks in the casing congeals at such a rate that the said leaks are automatically sealed substantially without any loss of insulating material.

The invention offers the advantage that the said danger is avoided and that moreover a less perfect and consequently simpler seal of the casing may be initially provided.

The insulating material of the invention may be insulating air-drying lacquers, comprising for example as a base, an air-drying oil.

By way of example we quote below a composition especially suited for use in carrying out the invention. A mixture of 1 part of colophony and 1 part of dammar resin is heated at a temperature of about 300° C. The greater part of the gaseous products thus produced is separated by distillation and to the mixture there is added sufficient zinc oxide to neutralise the free acids. To the molten resin mixture thus obtained there is added a mixture of 4½ parts of wood oil and 1½ parts of linseed oil, which resulting mixture is then maintained at a temperature of 270° C. for about half an hour, and subsequently cooled.

For the purpose of the invention automatic sealing is to be understood to mean that there occurs substantially no loss of insulating material when the viscous material is exposed to air at 20° C. under a hydrostatic pressure of 4 grs. per square cm. through an aperture having a length of 1 cm. and a diameter of 0.25 mm.

The invention is particularly important in

connection with transformers which are used for generating very high voltages since, as is well-known, a liquid or semi-liquid impregnating material is generally more resistant against such high voltage in the course of time than a solid or a more or less brittle material.

When carrying the invention into practice the form of wire insulation used in the electrical apparatus is to be taken into account and liquids, particularly aromatic liquids, having a high dissolving power should generally be avoided if the electrical apparatus contains the usual forms of enamel wire.

In the single figure of the drawing forming part of the specification there is shown, partly in cross-sectional view, a transformer assembly comprising a metal container 10, a transformer 11 (shown in block form) and an electrically insulating liquid 12 filling the container and impregnating and surrounding the transformer. The insulating liquid 12, consisting for example, of the material above specifically described, has the property of congealing when exposed to air at such a rate as to automatically seal leaks, for example, as shown at 13, which occur in the container.

The windings of the transformer are connected to insulated bushings 14 secured in the cover of the container and by which external electrical connections may be made to the transformer.

What we claim is:

Electrical apparatus comprising a container subject to leaks, an electrical insulating liquid within the container, and an electrical device immersed in the liquid, said liquid consisting of substantially a mixture of the reaction product of approximately one part colophony and one part dammar resin, zinc oxide in an amount sufficient to neutralize the free acids of said reaction product and a mixture of approximately four parts wood oil and one part linseed oil, said liquid having the property of congealing when in contact with air at such a rate as to automatically seal the container leaks without any substantial loss of the insulating liquid.

GILLES HOLST.  
JOHANNES HOCKSTR...